

## UNITED STATES PATENT OFFICE

SIEGMUND LOEWE, OF BERLIN, GERMANY, ASSIGNOR TO RADIO CORPORATION OF AMERICA, A CORPORATION OF DELAWARE

## PROCESS OF MAKING ELECTRON DISCHARGE DEVICES

No Drawing. Application filed August 21, 1926, Serial No. 130,769, and in Germany August 25, 1925.

This invention relates to a process of making vacuum tubes and more particularly vacuum tubes having highly emissive qualities. In accordance with this invention a vaporizable metal is dispersed in very small quantities in a highly evacuated tube, so that no mirror will be formed upon the bulb and the transparency of the latter will be essentially preserved. According to this invention, furthermore, the vaporizable metal, such as magnesium, is preferably alloyed with the surface of a nonvaporizable body, which while being heated will give off only minute quantities of magnesium. A further feature of this invention consists in, that the vaporizable metal is made to form a part of the system of the tube, preferably the anode. Further features of this invention consist in the manner of alloying said nonvaporizable metal body with the vaporizable metal.

According to the usual practice, in certain kinds of vacuum tubes highly emissive qualities are obtained by having, for instance, an ordinary tube with an incandescent cathode of thoriated tungsten first evacuated as fully as possible and thereupon subjected to a process, which consists in the dispersion of a metal, such as for instance magnesium. Ordinarily such tubes are rendered highly emissive after being subjected for some time to a process of formation or activation by keeping the cathode for some time in incandescent condition with or without applying the anode voltage thereto. The glass-bulbs of such tubes will seem from their exterior to have a mirror inside the bulb, due to the dispersion or vaporization of the metal. This metallic mirror which is deposited on the interior surface of the glass-bulb results in a number of grave disadvantages.

In the first place it will be impossible or at least very difficult, on account of the presence of such a mirror, to see whether the tube is in condition for operation, that is whether the cathode is in incandescent condition, and in the second place, the interior metallic mirror will reflect the heat to such a considerable extent that the entire heat carried off by radiation will be passed through those parts of the bulb which are free of the mirror. Or-

dinarily this is only that portion at which the electrodes extend through the wall of the tube, that is to say, the stem press of the tube. These portions, which permit the heat to be carried to the outside of the tube, will therefore become heated by absorption of heat. Among other things, in this case there is the disadvantage that an evolution of gas will take place which prevents the proper formation of the cathode, as has been proven by experiments; furthermore a really stationary condition of operation will be brought about only after a very long time, that is until the temperature conditions have become stationary. Therefore, a continuous slow variation of the operating conditions will take place as long as the temperature conditions have not become stationary.

This invention has for its object, to utilize all advantages which are connected with the dispersion or evaporation of the metal, and at the same time avoid the above-mentioned disadvantages.

Experiments have shown that an extremely small vaporization of magnesium will be sufficient to permit the formation or activation of the cathode to its full extent. It appears that—in contra-distinction to the now prevailing opinion—the process of formation or activation is even favourably affected by especially weak metal deposits. According to the known processes, therefore, unnecessarily large quantities of metal have apparently been used for the process of dispersion, which on account of its useless surplus in the depositing of metal has resulted in the above-mentioned disadvantageous features. However, in carrying out the process according to this invention, it is necessary to proceed in such a manner that the dispersion of the metal, although taking place only to a very small extent, is not started until a high vacuum has been obtained by carefully degassing the metal parts of the tube.

It has further been found that it is advantageous to provide metal parts within the tube, such as for instance parts of nickel, which are superficially alloyed with magnesium or another vaporizable metal. This

mode of operation, however, represents only one form of the process according to this invention. This alloy is made in such a manner that nickel, for instance in form of a sheet, is brought to incandescence in a vacuum furnace and that magnesium vapors are conveyed past the nickel body. The alloy which is thus obtained from nickel and magnesium has the property of again decomposing in the vacuum into its constituents. A peculiar feature has been found to exist with this process, viz., that the decomposing of the alloy takes place at temperatures which increase with the degree of vacuum and the temperature employed during the process of forming the alloy. In addition, during this decomposition the quantities of magnesium which are again given off will be in inverse proportion to the degree of vacuum and the temperature employed during the process of forming the alloy. By properly choosing the conditions, therefore, one will be enabled to produce alloys which will again give off minute quantities of magnesium in the vacuum tube only when in a condition of incandescence or at very high temperature. Nickel-magnesium alloys which are thus produced are extremely well suited for the purpose aimed at by this invention.

If, for instance, the anode of a rectifying, amplifying or oscillating tube is made of a nickel sheet which is alloyed in the aforescribed manner with difficultly volatizable magnesium, a high temperature will be required in order to drive out minute quantities of magnesium from the body of the anode. These minute quantities of magnesium will hardly have an effect upon the transparency of the glass-bulb and there will at most be a very slight blackening of the glass, but in no case is an opaque metallic mirror formed thereupon. The glass-wall of a tube which is made in this manner will still be almost as permeable for heat as a tube without mirror, while experiments have shown that the formation or activation of the cathode may be brought about in such case rather more easily than with tubes having the usual strong mirror.

The magnesium, which had been employed in the experiments, consisted of the ordinary chemically pure magnesium obtainable on the market, said magnesium having contained also admixtures of other substances, such as for instance, calcium.

It has further been found, that in the same manner tungsten as well as tantalum and molybdenum sheets may be alloyed with magnesium, so that one will be enabled to likewise produce electrodes having a high melting point, which may be used for high-powered tubes serving for transmitting purposes.

It is furthermore of especial importance,

that also Roentgen-tubes with cathodes of highly emissive qualities may be made in the aforescribed manner, because the hardly visible deposit which is produced upon the glass-wall will in no way obstruct the passage of Roentgen rays and also fully avoid the production of heat due to the passage of the rays through glass-walls having a heavy mirror.

I claim:

1. The method of producing an anode for an electron discharge tube which comprises shaping a sheet of metal to the form of an anode, heating said sheet to a temperature slightly higher than the temperature attained by said anode under normal operating conditions of the electron discharge tube, and exposing said sheet of metal while so heated to vaporized magnesium at a pressure no greater than the normal pressure in the electron discharge tube and thereby forming on said anode a coating of an alloy of said metal and magnesium which decomposes very slowly during normal operation of the electron discharge tube.

2. The method of producing an anode for an electron discharge tube which comprises shaping a sheet of metal to the form of an anode, exposing a sheet of nickel to vaporized magnesium at a pressure no greater than the pressure in the electron discharge tube and heating said sheet while so exposed to a temperature slightly higher than the normal operating temperature of said anode and thereby forming a surface alloy of nickel and magnesium which decomposes very slowly under normal operation of said anode in the electron discharge tube.

In testimony whereof I have affixed my signature.

SIEGMUND LOEWE.

70

75

80

85

90

95

100

105

110

115

120

125

130